# EUROPEAN PATENT SPECIFICATION

(11) **EP 2 992 143 B1**
(45) Date of publication and mention of the grant of the patent: **19.04.2017**
(21) Application number: 14730836.5
(22) Date of filing: 11.06.2014
(51) Int. Cl.: D21H 25/04, D21H 19/38, D21H 19/40, D21H 19/66

(54) **PAPER MATERIAL HAVING HOLOGRAPHIC AND PEARLESCENT METALLIC EFFECTS AND THE MANUFACTURING PROCESS THEREOF**
PAPIERMATERIAL MIT HOLOGRAFISCHEN UND PERLGLÄNZENDEN METALLIC-EFFEKTEN SOWIE HERSTELLUNGSVERFAHREN DAFÜR
MATÉRIAU DE PAPIER COMPORTANT DES EFFETS HOLOGRAPHIQUES ET MÉTALLIQUES PERLÉS ET SON PROCÉDÉ DE FABRICATION

(30) Priority: 13.06.2013 IT MI20130979
(43) Date of publication of application: 09.03.2016
(73) Proprietor: GRUPPO CORDENONS S.p.A., 20145 Milano (IT)
(72) Inventor: MONACELLI, Luca, I-33170 Pordenone (IT); GILBERTI, Ferruccio, I-20121 Milano (IT)
(74) Representative: Rapisardi, Mariacristina
(86) International application number: PCT/EP2014/062145
(87) International publication number: WO 2014/198780

(56) References cited:
- EP-A1- 2 520 709
- EP-A2- 1 762 656
- WO-A1-02/12621
- WO-A1-95/06568
- WO-A1-2004/099500
- WO-A1-2010/076392
- US-A- 4 409 280
- US-A- 5 571 557

## Description

The present invention relates to a paper material (paper/pasteboard) having holographic and pearlescent metallic effects and to the manufacturing process thereof.

More precisely, owing to a specially-formulated pulp and a specific treatment of the surface, the paper material of the invention exhibits a particular three-dimensional pearlescent effect.

In the paper sector, there is a constant, ongoing search for new types of paper with particular appearances and/or finishes, especially papers intended for packing, packaging, for realizing illustrative material, for quality printing, etcetera.

It , however, that the achievement of special effects jeopardizes other characteristics of the paper, such as printability.

EP 2520709 A1, WO2004/099500 A1, WO02/12621 A1 and US 5 571 557 A disclose a paper material according to the preamble of claim 1.

It is an object of the present invention to provide a paper material that has an optical effect differing from that of conventional paper materials and that is at the same time printable with high printing quality.

The present invention relates therefore to a paper material and the manufacturing process thereof as defined in appended claims 1 and 8, respectively.

Preferred embodiments of the paper material and of the manufacturing process thereof are defined in the dependent claims. The invention provides therefore a pearlescent paper material (paper/pasteboard) having a three-dimensional holographic effect, owing to a specially-formulated pulp and a specific treatment of the surface, and to a production method that enables orientation of the pearlescent pigments according to a predetermined design.

The paper material of the invention also proves to be perfectly printable with high printing quality and makes it possible to achieve particular graphic effects that are difficult to achieve with conventional coated paper stocks.

More specifically, the paper material of the invention comprises a support base made up of a mixture of cellulose fibres and containing at least one polymeric substance suitable for conferring strength (dry or wet) to the mixture of fibres, and an inorganic filler suitable for conferring good machinability characteristics to the material.

The polymeric substance included in the support base preferably comprises one or more colophony-based and/or alkyl-ketene-dimer-based and/or acetylsuccinic-acid-based and/or epichlorohydrin-based resins, and/or modified starches; the inorganic filler is a mineral filler comprising one or more substances selected from the group constituted by carbonates, kaolins, talc and mixtures thereof.

The support base has at least one surface (face) that is treated with at least one surface adhesive, preferably an adhesive based on starch and/or polyvinyl alcohol and/or acrylic, polyurethane and/or styrene-butadiene polymers.

Moreover, the paper material of the invention is provided with a coating applied on the surface treated with the adhesive (clearly, both surfaces of the paper material can be treated and provided with coating).

Specifically, the coating comprises one or more binder polymers (for example polyurethane- and/or silicone-based polymers, and/or acrylic, styrene-butadiene, polyvinyl acetate, polyvinyl alcohol polymers, and similar polymers) and/or waxes, mixed with pigments, preferably magnetic or diamagnetic metallic pearlescent and/or magnetic or diamagnetic non-metallic pearlescent pigments of various colours and particle sizes.

These pearlescent pigments are sensitive to a magnetic field so as to be oriented according to a predefined design.

The grammage of the paper material preferably ranges between approximately 90 and approximately 350 g/m²; the amount of coating spread on each face ranges between about 5 and 20 g/m²; and the amount of polymer in the coating is preferably within the range of 5% to 100% with respect to the pigments.

The coating can be coloured and/or spread on a coloured support base; preferably, paste stains and organic or inorganic pigments are used.

In this manner, through the combined effect of the composition of the support base, the pigments and the surface treatment, the paper material exhibits a holographic pearlescent effect with various colours.

Both faces of the support base can clearly be treated in the same manner.

In accordance with a further aspect of the present invention, the paper material described hereinabove is realized using the method as described below.

At first the support base is realized, using a substantially known technique for making paper, for example on a paper machine for manufacturing paper.

Essentially, an aqueous pulp of cellulose fibres and containing the polymeric substance (colophony-based and/or alkyl-ketene-dimer-based and/or acetylsuccinic-acid-based and/or epichlorohydrin-based resins, and/or modified starches) and the inorganic filler (carbonates, kaolins, talc, etcetera) is prepared. The water is then removed from the pulp so as to form the support base of the paper material.

This is followed by a step of treating the surface of one or both faces of the support base with an aqueous solution of surface adhesive, for example composed of a 10% by weight aqueous solution of starch, and/or 5% by weight acrylic adhesive, or similar adhesives based on polyvinyl alcohol and/or acrylic, polyurethane and/or styrene-butadiene polymers.

Following treatment of the surface with adhesive, the method comprises then a step of smoothing the support base, in which the support base is smoothed up to Bendtsen (ISO 2494) smoothness values of less than about 50 ml/min and preferably of less than about 30 ml/min and indicatively of about 20 ml/min.

The previously described step of applying the coating follows.

Application of the coating preferably occurs by means of spreading using air-knife and/or smoothing-blade technology, rotooffset, rotographic and flexographic techniques.

The coating thus applied is then subjected to a magnetic field varying in intensity and applied preferably by means of a solenoid or a magnet structured so as to orient the pearlescent pigments according to different types of designs; this solenoid can be rotating at the same speed as the paper, oscillating on the plane x and/or fixed.

There is then a step of drying the coating, performed in an infrared and/or hot-air oven at a temperature ranging between approximately 100 °C and approximately 180 °C and with an oven residence time ranging between 0.5 and 4 minutes.

Lastly, the method comprises a step for mechanical treatment of the surface provided with the coating, in particular a smoothing step and/or an embossing step.

It should be observed that the wastewater and coating waste resulting from the production process in a paper mill must be treated for purification purposes.

Pollutants are present in various forms in the wastewaters of paper mills: sedimentable substances such as fibre, mineral fillers, etc., colloidal substances, and dissolved substances such as inorganic salts (chlorides, sulphates, etc.).

Purification of the wastewater of paper mills occurs by means of various steps.

### Step 1: Physico-chemical purification system

This step comprises the following treatments.

### Grit removal

The first treatment applied for purification of the wastewater consists of grit removal, which is used for elimination of coarse solids such as paper, plastic, wood, etc., i.e. materials of large sizes capable of creating blockage in some units in the plant.

### Equalization

The wastewater coming from the machines and wastewater coming from the coating treatment are conveyed into the inlet tank for the purpose of making the concentration of polluting agents constant so as to optimize the subsequent treatments.

The wastewater in the equalization tank is constantly agitated so as to prevent sedimentation of pollutant substances on the bottom.

### Sediment flotation

This purification step takes place in the "sediment flotation unit" where sedimentation and flocculation of the solid substances dissolved in the wastewater take place.

### Sedimentation

The process of sedimentation is achieved by keeping the water in the sediment flotation unit in a quiet stage and thus sedimentation of the materials that are denser than the water takes place.

The force of gravity is used in the sedimentation step to separate the solid particles of a greater density than that of the water from the water.

The deposited materials consist of sand, inorganic oxides and biological sludge. The sand settles on the bottom of the sediment flotation unit spontaneously, whereas the inorganic oxides and biological sludge are made to settle by adding chemical reagents such as alum and polyelectrolytes.

### Coagulation

The colloidal substances are not completely separated from the water by the sedimentation process.

Cationic inorganic reagents that enable the formation of small flocs are added to coagulate the colloids.

### Flocculation

Flocculation is the agglomeration of destabilized particles into flocs.

With the addition of a flocculant such as a polyelectrolyte, the flocs increase in size and settle or float according to their nature.

### Flotation

The particles of a density approximately equal to that of the water are separated by means of the flotation process.

This process is based on the capacity of certain particles to bind to the gas bubbles, normally air bubbles, so as to form a gas-particle system having a density lower than the density of the water.

In this manner, the particles rise towards the surface of the water.

Sedimented sludge is removed by a doctor blade on the bottom of the sediment flotation unit, whereas the sludge flocs are removed by a screw.

The sediment and flocs are collected in two vats for subsequent pressing.

The purified water is collected through a drain placed at the centre of the tank and sent to the equalization tank of the biological purification system.

### Step 2: Biological System

This step comprises the following treatments.

### Equalization

After passing through the Physico-chemical purification system, the wastewater is sent to the equalization tank of the biological purification system.

The biological purification system utilizes a culture of aerobic bacteria that make it possible to lower the COD and remove the surfactants present in the wastewater.

An optimal pH level for the growth of the bacteria ranges between 6.5 and 7.5. Bacteria need organic nutrients for growth and multiplication. The biological

purification processes use the metabolism of the bacteria for the transformation of the organic substances.

The bacteria use part of the organic substances dissolved in the wastewater for their development, transforming them into active sludge. In particular, an aerobic bacterial culture is capable of transforming the carbon present in solution into new tissue and into carbon dioxide.

The high concentrations of bacteria present in the oxidation tank are possible owing to the recycling of active sludge by DAF.

### Oxidation

The aerobic bacteria use the oxygen dissolved in the water and to achieve optimal activity, oxygen is added to the water in the oxidation tank.

The organic substances and surfactants are removed in the oxidation tank.

### Removal of Nitrogen and Phosphorus

Nitrogen is present principally in the form of ammonia initially bound in complex organic molecules.

Ammonia nitrogen can be biologically oxidized to nitrites:

2NH₃ + 3O₂ → 2NO₂⁻ + 2H⁺ + 2H₂O

Lastly, the nitrites can be oxidized further, biologically again, to nitrates:

2NO₂⁻ + O₂ + → 2NO₃⁻

The overall transformation is as follows:

NH₃ + 2O₂ → NO₃⁻ + H⁺ + H₂O

The nitrogen tends to leave the liquid medium as nitrogen gas:

2NO₃⁻ → 3O₂ + N₂

Phosphorus is necessary for the construction of the cell membrane of the aerobic bacteria, and therefore in its absence, it must be added to the water entering the purification plant. If in excess, however, it is removed by chemical precipitation processes, using coagulation/flocculation products.

Two typical precipitation reactions with aluminium sulphate and with lime, which are effective mainly on orthophosphates, are as follows:

Al₂(SO₄)₃ +14H₂O + 2PO₄³⁻ → 2AlPO₄(s) + 2SO₄²⁻ + 14H₂O

3Ca(OH)₂ + 2PO₄³⁻ → Ca₃(PO₄)₂ (s) + 6OH⁻

The separation of the organic sludge from the purified wastewater subsequently occurs in the DAF flotation tank (dissolved air flotation).

Binding to the air bubbles, the sludge rises by flotation to the surface and the sludge is recovered by an Archimedean screw recycling in the oxidation tank.

Excess sludge is sent to a sludge press.

### Filtration

Before entering a drainage channel, the waters are filtered by eight sand filters and passed into the sedimentation tank for purified water so as to eliminate the last residues of fibre.

It is also understood that modifications and variations may be made in the described and illustrated paper material and manufacturing method thereof without departing from the scope of the invention as defined in the appended claims.

## Claims

1. A paper material comprising a support base, made up of a mixture of cellulose fibres containing at least one polymeric substance suitable for conferring strength to the mixture of fibres, and an inorganic filler suitable for conferring good workability characteristics to the mixture, said paper material having at least one external surface treated with at least one surface adhesive and whereon at least one coating is applied, **characterized in that** said coating comprises pearlescent pigments sensitive to a magnetic field applied to orient said pearlescent pigments according to a predefined design.

2. The paper material according to claim 1, **characterized in that** said coating comprises one or more binder polymers and/or waxes, mixed with pigments.

3. The paper material according to any one of claims 1 or 2, **characterized in that** said pearlescent pigments comprise magnetic or diamagnetic metallic pigments and/or magnetic or diamagnetic non-metallic pigments.

4. The paper material according to any one of the preceding claims, **characterized in that** said polymeric substance included in the said support base comprises one or more colophony-based and/or alkyl-ketene-dimer-based and/or acetylsuccinic-acid-based and/or epichlorohydrin-based resins, and/or modified starches.

5. The paper material according to any one of the preceding claims, **characterized in that** said inorganic filler included in the said support base is a mineral filler and comprises one or more substances selected from the group constituted by carbonates, kaolins, talc and mixtures thereof.

6. The paper material according to any one of the preceding claims, **characterized in that** said surface adhesive is an adhesive based on starch and/or polyvinyl alcohol and/or acrylic, polyurethane and/or styrene-butadiene polymers.

7. The paper material according to any one of the preceding claims, **characterized in that** said coating-binding polymers comprise polyurethane-based, acrylic-based, polyvinyl- alcohol-based, styrene-butadiene-based and/or silicone-based polymers.

8. A method for manufacturing the paper material, comprising the steps of:
- preparing an aqueous pulp of cellulose fibres containing at least one polymeric substance suitable for conferring strength to the mixture of fibres, and an inorganic filler suitable for conferring good workability characteristics to the mixture;
- removing water from the aqueous pulp of fibres so as to form a support base of the paper material;
- treating at least one external surface of the support base with at least one surface adhesive, in such a manner as to confer proper water penetration to the paper material, which is indispensable for the coating step, **characterized in that** it further comprises the steps of:
- applying a coating to the surface treated with the adhesive, said coating comprising one or more binder polymers and/or waxes, mixed with pearlescent pigments sensitive to a magnetic field;
- applying a magnetic field so as to orient the pearlescent pigments according to a predefined design.

9. The manufacturing method according to claim 8, **characterized in that** the application of the magnetic field is realized by means of a static and/or dynamic and/or oscillating and/or varying-intensity magnetic field applied by means of a solenoid or a magnet.

10. The manufacturing method according to any one of claims 8 or 9, **characterized in that** following treatment of the surface with the adhesive and prior to application of the coating, it comprises a step for smoothing the support base, wherein the support base is smoothed up to Bendtsen ISO 2494 smoothness values of less than 50 ml/min, preferably of less than 30 ml/min and indicatively of about 20 ml/min.

11. The manufacturing method according to any one of claims 8 to 10, **characterized in that** the step for application of the coating takes place by blade-coating.

12. The method according to any one of claims 8 to 11, **characterized in that** it comprises a step for drying the coating, which is performed in an infrared and/or hot-air oven at a temperature ranging between approximately 100 °C and approximately 180 °C and with an oven time ranging between 0.5 and 4 minutes.

13. The method according to any one of claims 8 to 12, **characterized in that** it comprises a step for mechanical treatment of the surface provided with the coating, in particular a smoothing step and/or an embossing step.

## Patentansprüche

1. Papiermaterial, das eine Trägerbasis umfasst, bestehend aus einer Mischung aus Zellulosefasern, enthaltend mindestens eine Polymersubstanz, geeignet die Mischung aus Fasern zu stärken und einen anorganischen Füllstoff, geeignet der Mischung gute Verarbeitbarkeitseigenschaften zu verleihen, wobei das Papiermaterial mindestens eine externe Oberfläche aufweist, die mit mindestens einem Flächenklebstoff behandelt wird und worauf mindestens eine Beschichtung aufgetragen ist, **dadurch gekennzeichnet, dass** die Beschichtung Perlglanzpigmente umfasst, die empfindlich auf ein magnetisches Feld sind, das angewendet wird, um die Perlglanzpigmente nach einem vorgegebenen Design zu orientieren.

2. Papiermaterial nach Anspruch 1, **dadurch gekennzeichnet, dass** die Beschichtung ein oder mehrere Bindemittelpolymere und/oder Wachse, gemischt mit Pigmenten, umfasst.

3. Papiermaterial nach einem der Ansprüche 1 oder 2, **dadurch gekennzeichnet, dass** die Perlglanzpigmente magnetische oder diamagnetische Metallpigmente und/oder magnetische oder diamagnetische nicht-metallische Pigmenten umfassen.

4. Papiermaterial nach einem der vorhergehenden Ansprüche, **dadurch gekennzeichnet, dass** die Polymersubstanz, die in der Trägerbasis einbezieht ist, ein oder mehrere Kolophonium-basierte und/oder Alkyl-Ketene-Dimer-basierte und/oder Acetylsuccinat-Säurebasierte und/oder Epichlorhydrin-basierte Harze und/oder modifizierte Stärken umfasst.

5. Papiermaterial nach einem der vorhergehenden Ansprüche, **dadurch gekennzeichnet, dass** der anorganische Füllstoff, der in der Trägerbasis einbezieht ist, ein Mineralfüllstoff ist und eine oder mehrere Substanzen umfasst, die aus der Gruppe ausgewählt werden, die aus Karbonaten, Kaolinen, Talkum und deren Mischungen besteht.

6. Papiermaterial nach einem der vorhergehenden Ansprüche, **dadurch gekennzeichnet, dass** der Flächenklebstoff ein Klebstoff auf Basis von Stärke und/oder Polyvinylalkohol und/oder Acryl-, Polyurethan- und/oder Styrol-Butadien-Polymere ist.

7. Papiermaterial nach einem der vorhergehenden Ansprüche, **dadurch gekennzeichnet**, das die beschichtenden-bindenden Polymere Polyurethan-basierte, Acryl-basierte, Polyvinyl-Alkohol-basierte, Styrol-Butadien-basierte und/oder Silikon-basierte Polymere umfassen.

8. Verfahren zur Herstellung vom Papiermaterial, umfassend die Schritte:
- Vorbereiten eines wässrigen Breis aus Zellulosefasern, enthaltend mindestens einen Polymerstoff, geeignet die Fasermischung zu stärken, sowie einen anorganischen Füllstoff, geeignet der Mischung gute Verarbeitbarkeitseigenschaften zu verleihen,
- Beseitigen des Wassers aus dem wässrigen Brei aus Fasern, um eine Trägerbasis des Papiermaterials zu bilden;
- Behandeln mindestens eine externe Oberfläche der Trägerbasis mit mindestens einem Flächenklebstoff, sodass richtiges Wassereindringen dem Papiermaterial verleiht wird, welches unverzichtbar für den Beschichtungsschritt ist, **dadurch gekennzeichnet, dass** es die Schritte weiterumfasst:
- Auftragen einer Beschichtung auf der Oberfläche, die mit dem Klebstoff behandelt wird, wobei die Beschichtung ein oder mehrere Polymerbindemittel und/oder Wachse umfasst, die mit Perlglanzpigmenten gemischt werden, die empfindlich auf ein Magnetfeld sind;
- Anwenden eines Magnetfeldes, um die Perlglanzpigmente nach einem vordefinierten Design zu orientieren.

9. Herstellungsverfahren nach Anspruch 8, **dadurch gekennzeichnet, dass** die Anwendung des Magnetfeldes mittels eines statischen und/oder dynamischen und/oder oszillierenden und/oder unterschiedlich intensiven Magnetfeldes erfolgt, das mittels eines Magnetventils oder eines Magnets angewendet wird.

10. Herstellungsverfahren nach einem der Ansprüche 8 oder 9, **dadurch gekennzeichnet, dass** nach der Behandlung der Oberfläche mit dem Klebstoff und vor dem Auftragen der Beschichtung, einen Schritt zum Glätten der Trägerbasis umfasst, wobei die Trägerbasis bis Bendtsen ISO 2494 Glättewerte von weniger als 50 ml/min, vorzugsweise von weniger als 30 ml/min und als Richtwert von etwa 20 ml/min geglättet wird.

11. Herstellungsverfahren nach einem der Ansprüche 8 bis 10, **dadurch gekennzeichnet, dass** der Schritt zum Auftragen der Beschichtung durch Klinge-Beschichtung erfolgt.

12. Verfahren nach einem der Ansprüche 8 bis 11, **dadurch gekennzeichnet, dass** es einen Schritt zur Trocknung der Beschichtung umfasst, die in einem Infrarot-und/oder Heißluft-Ofen bei einer Temperatur im Bereich von ca. 100 °C bis ca. 180 °C und mit einer Ofenzeit im Bereich zwischen 0,5 und 4 Minuten durchgeführt wird.

13. Verfahren nach einem der Ansprüche 8 bis 12, **dadurch gekennzeichnet, dass** es einen Schritt der mechanischen Bearbeitung der Oberfläche, versehen mit der Beschichtung, insbesondere einen Schritt zum Glätten und/oder einen Schritt zum Prägen, umfasst.

## Revendications

1. Matériau de papier comprenant une base de support composée d'un mélange de fibres de cellulose contenant au moins une substance polymère pouvant conférer une solidité au mélange de fibres, et une charge inorganique pouvant conférer de bonnes caractéristiques de maniabilité au mélange, ledit matériau de papier comportant au moins une face externe traitée avec au moins un adhésif de surface et sur laquelle est appliqué au moins un couchage, **caractérisé en ce que** ledit couchage comprend des pigments perlés sensibles à un champ magnétique appliqué pour orienter lesdits pigments perlés selon un motif prédéfini.

2. Matériau de papier selon la revendication 1, **caractérisé en ce que** ledit couchage comprend un ou plusieurs polymères liants et/ou cires, mélangés(ées) aux pigments.

3. Matériau de papier selon l'une quelconque des revendications 1 ou 2, **caractérisé en ce que** lesdits pigments perlés comprennent des pigments métalliques magnétiques ou diamagnétiques et/ou des pigments non métalliques magnétiques ou diamagnétiques.

4. Matériau de papier selon l'une quelconque des revendications précédentes, **caractérisé en ce que** ladite substance polymère incluse dans ladite base de support comprend une ou plusieurs résines à base de colophane et/ou de dimère d'alkyl-cétène et/ou d'acide acétylsuccinique et/ou d'épichlorhydrine, et/ou d'amidons modifiés.

5. Matériau de papier selon l'une quelconque des revendications précédentes, **caractérisé en ce que** ladite charge inorganique incluse dans ladite base de support est une charge minérale et comprend une ou plusieurs substances sélectionnées dans le groupe composé de carbonates, kaolins, talc et leurs mélanges.

6. Matériau de papier selon l'une quelconque des revendications précédentes, **caractérisé en ce que** l'adhésif de surface est un adhésif à base d'amidon et/ou d'alcool polyvinylique et/ou d'acrylique, de polyuréthane et/ou de polymères butadiène-styrène.

7. Matériau de papier selon l'une quelconque des revendications précédentes, **caractérisé en ce que** lesdits polymères liants-de couchage comprennent des polymères à base de polyuréthane, d'acrylique, d'alcool polyvinylique, de butadiène-styrène et/ou de silicone.

8. Procédé de fabrication de matériau de papier, comprenant les étapes de :
- préparer une pâte aqueuse de fibres de cellulose contenant au moins une substance polymère pouvant conférer une solidité au mélange de fibres, et une charge inorganique pouvant conférer de bonnes caractéristiques de maniabilité au mélange ;
- retirer l'eau de la pâte aqueuse de fibres de manière à former une base de support du matériau de papier ;
- traiter au moins une face externe de la base de support avec au moins un adhésif de surface de manière à conférer au matériau de papier une absorption d'eau appropriée étant indispensable pour l'étape de couchage, **caractérisé en ce qu'**il comprend de plus les étapes de :
- appliquer un couchage à la face traitée avec l'adhésif, ledit couchage comprenant un ou plusieurs polymères liants et/ou cires mélangés(ées) aux pigments perlés sensibles à un champ magnétique ;
- appliquer un champ magnétique de manière à orienter les pigments perlés selon un motif prédéfini.

9. Procédé de fabrication selon la revendication 8, **caractérisé en ce que** l'application du champ magnétique est réalisée au moyen d'un champ magnétique statique et/ou dynamique et/ou oscillant et/ou d'intensité variable appliqué au moyen d'un solénoïde ou d'un aimant.

10. Procédé de fabrication selon l'une quelconque des revendications 8 ou 9, **caractérisé en ce que** après le traitement de la surface avec l'adhésif et avant l'application du couchage, il comprend une étape consistant à satiner la base de support, dans lequel la base de support est satinée jusqu'à des valeur de rugosité Bendtsen ISO 2494 inférieures à 50 ml/min, de préférence inférieures à 30 ml/min et à titre indicatif d'environ 20 ml/min.

11. Procédé de fabrication selon l'une quelconque des revendications de 8 à 10, **caractérisé en ce que** l'étape consistant à appliquer le couchage se déroule par couchage par lame.

12. Procédé selon l'une quelconque des revendications de 8 à 11, **caractérisé en ce qu'**il comprend une étape de séchage du couchage étant réalisée dans un four à infrarouges et/ou un four à air chaud à une température comprise approximativement entre 100 et 180 °C pendant une durée comprise entre 30 secondes et 4 minutes.

13. Procédé selon l'une quelconque des revendications de 8 à 12, **caractérisé en ce qu'**il comprend une étape de traitement mécanique de la face pourvue du couchage, en particulier une étape de satinage et/ou une étape de gaufrage.
